

Patented July 1, 1924.

1,500,026

## UNITED STATES PATENT OFFICE.

EDWARD MENDELSON, OF NEW YORK, N. Y., ASSIGNOR TO LANSDALE SILK HOSIERY CO., INC., OF LANSDALE, PENNSYLVANIA, A CORPORATION OF PENNSYLVANIA.

### METHOD OF TREATING SILK STOCKINGS.

No Drawing.

Application filed April 4, 1924. Serial No. 704,292.

To all whom it may concern:

Be it known that I, EDWARD MENDELSON, a citizen of the United States, and resident of New York, in the county of New York 5 and State of New York, have invented certain new and useful Improvements in Methods of Treating Silk Stockings, of which the following is a specification.

The main object of this invention is to 10 give to thin silk stockings a more sheer appearance and at the same time to increase the strength and durability. By the use of my improved process various other important objects and advantages are secured, 15 certain of which will be hereinafter referred to.

Although my invention might be employed in connection with silk fabrics and for garments other than stockings, it is particularly applicable to very thin or sheer silk stockings. In carrying out my invention the stockings are first thoroughly wet or soaked in cold water containing alum. I preferably used the ammonium 25 alum although potassium alum might be employed. The amount of alum employed is preferably about five per cent by weight of the water. After the alum solution has had sufficient time to thoroughly permeate the 30 threads, the stockings are removed and treated with a soap solution; the percentage of soap in the solution is probably about  $\frac{1}{2}$  of 1%. The soap reacts with the alum to form an insoluble metallic soap within and 35 around the fibers forming the silk threads.

As a result of this treatment, the fibres going to make up the threads are brought in more compact relationship; the loose fibre ends are caused to adhere to the body portion of the threads and the threads are thereby reduced in effective size and made harder and more compact. The compacting of the fibres also tends to increase the strength of the individual threads and permits them to slide over each other during 40 the bending or stretching of the fabric. It also increases the elasticity. The elimination of the loose or fluffy ends of the fibres also reduces the liability of the fabric being torn in case any sharp object rubs against 45

it, or where under strain as for instance, at the garter clasps. The insoluble metallic soap forms a very thin coating over the threads which is not removed by later washings and therefore the dye in the threads is 55 preserved and there is less liability of fading by repeated washings. The coating also protects the threads against the action of perspiration.

I am aware that it has been proposed to 60 deposit insoluble metallic soap on cloth to render the same waterproof, but in my improved process, the sheer silk is rendered even less water-proof because the individual threads are rendered more compact and of 65 smaller effective size, and the openings between the threads are thereby enlarged rather than closed up or plugged. This is important in connection with thin silk stockings, as sheer appearance and ventilation are both desired. 70

Having thus described my invention, what I claim as new, and desire to secure by Letters Patent, is:

1. The process of treating silk stockings 75 to render them stronger and more sheer in appearance, which consists in subjecting them to the action of an alum solution and thereafter subjecting them to the action of the soluble soap solution. 80

2. The process of treating silk stockings which consists in subjecting them to an action of solution containing approximately 5% of alum and thereafter subjecting them to an action of a solution containing approximately  $\frac{1}{2}$  of 1% of soap. 85

3. The herein described method of treating silk fabrics to increase the strength, durability and sheer appearance which consists in subjecting them to the action of relatively strong alum solution and thereafter subjecting them to the action of a relatively weak soluble soap solution, to harden and compact the threads and thereby increase the size of the apertures between the 90 threads. 95

Signed at New York, in the county of New York and State of New York, this third day of April, A. D. 1924.

EDWARD MENDELSON.